

## UNITED STATES PATENT OFFICE

1,993,396

## PROCESS OF DEWAXING MINERAL OILS

Harry T. Bennett, Tulsa, Okla., assignor to Mid-Continent Petroleum Corporation, Tulsa, Okla., a corporation of Delaware

No Drawing. Application January 9, 1930,  
Serial No. 419,747

9 Claims. (Cl. 196—19)

This invention relates to a process of removing wax from mineral oils, including petroleum products. More particularly it relates to a method for removing crystal-forming wax from petroleum products, especially lubricating oil.

When the wax exists in a petroleum oil in an amorphous state it can be readily removed by subjecting the oil to a centrifuging or similar operation. However, prior to this invention it has been extremely difficult if not impossible to remove the wax by centrifuging when it exists in a crystalline state. The methods used for removing amorphous wax would not satisfactorily remove crystal-forming wax, and attempts to remove crystal-forming wax by centrifuging have proved commercially unsatisfactory.

The object of this invention, therefore, is to economically remove the wax in a simple manner, regardless of its previous structure.

20 To the accomplishment of the foregoing object the invention comprises the steps hereinafter described and more particularly pointed out in the appended claims.

An approved method of carrying out this invention is set forth in detail in the following description, but it is to be understood that this specific disclosure does not set forth all of the several ways in which the principle of my invention may be used, and that various modifications conforming to the invention will be obvious to those skilled in this art.

In the following description the method is set forth as relating to lubricating oil. It is understood, however, that this invention is not limited to removing wax from lubricating oil because wax may be likewise removed from the other petroleum products.

I have found that the addition of a small quantity of soap, such as aluminum stearate which is substantially insoluble in water to the lubricating oil containing the crystal-forming wax will change the structure of the wax in such manner that the wax may be easily removed.

The amount of soap to be used will vary with the condition of the oil and the results desired. The amount, however, is preferably less than 2 percent of the weight of the mass and about 0.1 percent will, under ordinary conditions, give satisfactory results.

50 After the soap has been added to the oil it may or may not be necessary to stabilize the resultant mixture. If it is necessary to stabilize the mixture, the mixture may be heated to a temperature of about 350° F., or a separate stabilizing agent, such as benzyl alcohol may be used

so that the mixture containing the soap will not revert back to its original state, that is the wax will remain in such condition after treating that it can be easily removed from the oil.

The soap treated oil is then diluted with a low boiling point hydrocarbon, such as petroleum naphtha. However, any suitable diluent may be used. The amount of diluent is preferably approximately 40 to 80 percent of the volume of the resultant mixture. For example, there may be 10 sixty gallons of naphtha to every forty gallons of oil.

The resultant mixture is then chilled to a temperature of about 10° above zero to about 45° below zero F.

15 After chilling to the desired temperature, the mixture is subjected to centrifugal force and the wax removed.

The low boiling point hydrocarbon is then removed from the oil by distillation, or in any 20 other suitable manner.

The remaining soap and stabilizer, if a separate stabilizer is used, may then be either removed or left in the oil as desired.

In the foregoing process the wax, even though 25 it originally existed in a crystalline state, will be changed in structure, so that it can be easily removed by centrifuging in the manner ordinarily employed to remove amorphous wax. The advantages of such a process are readily apparent to those skilled in the art.

Petroleum oils containing crystal-forming wax are unsuited for use at a low temperature because the wax will harden and prevent satisfactory use of the products. Since this invention 35 shows how crystal-forming wax may be easily, quickly and effectively removed, which was previously thought commercially impossible, it is apparent that petroleum products which originally contained crystal-forming wax can now be 40 satisfactorily used at low temperatures.

This invention is especially valuable in treating lubricating oil distillates, as lubricating oils of this kind which have been subjected to vaporization and condensation usually contain the crystal-forming wax, while the wax in the oils remaining in the still is usually amorphous, or non-crystalline, when the oils are chilled. However, the invention may be used in treating any hydrocarbon oil containing crystal-forming wax.

45 As an example of one form of this invention, I will describe one method of treating an oil having a Saybolt universal viscosity of 55 at 210° F. and a pour point of 85° F. About 0.1 percent by weight of aluminum stearate was added to the 55

oil and the resultant mixture heated to 350° F. The resultant product was cooled to 100° F. and diluted with naphtha so that the resultant mixture contained 60 percent by volume of diluent. 5 The resultant mixture was then chilled to -20° F. and centrifuged to separate the mixture into two portions, i. e. oil and naphtha, and wax and naphtha. The naphtha was then removed from the oil by distillation. The finished oil had a 10 pour point of 25° F. and a Saybolt universal viscosity of 60 at 210° F.

I claim:

1. The method of removing crystal-forming wax from mineral oils, which comprises adding 15 aluminum stearate and naphtha to the oil to be treated, chilling the resultant mixture, subjecting the chilled mixture to centrifugal force to remove the wax, and removing the naphtha from the de-waxed oil.

20 2. The method of removing crystal-forming wax from petroleum oils which comprises adding aluminum stearate to the oil to be treated to render the wax removable at low temperatures, diluting the product with a quantity of petroleum 25 naphtha amounting to 40 to 80% of the volume of the resultant mixture, chilling said mixture, subjecting the same to centrifugal force to remove the wax, and removing said naphtha from said oil.

3. The method of removing crystal-forming 30 wax from lubricating oil which comprises adding aluminum stearate to the oil to be treated to facilitate removal of the wax at low temperatures, stabilizing the resultant mixture, diluting the oil with petroleum naphtha, chilling the mixture to 35 a temperature from 10° above zero F. to about 45° below zero F., subjecting the chilled mixture to centrifugal force to remove the wax, and removing said naphtha from said oil.

4. The method of removing crystal-forming 40 wax from lubricating oil which comprises preventing crystallization of the wax at low temperatures by adding less than 2% of aluminum stearate to the oil to be treated, stabilizing the resultant mixture by heating the same, diluting the 45 oil with a quantity of naphtha amounting to 40% to 80% of the volume of the resultant mixture, chilling said resultant mixture to a temperature from 10° above zero to about 45° below zero F., then subjecting the same to centrifugal force to 50 remove the wax, and removing said naphtha from said oil.

5. The method of removing crystal-forming wax from lubricating oil which comprises preventing crystallization of the wax at low temperatures by adding less than 2% of aluminum stearate to the oil to be treated, stabilizing the resultant mixture by heating the same to a temperature of about 350° F., diluting the oil with a quantity of petroleum naphtha amounting to 40% to 80% of the volume of the resultant mixture, chilling said mixture to a temperature from 10° above zero to about 45° below zero F., to remove the wax, and removing said naphtha and aluminum stearate from said oil.

6. The method of removing wax from petroleum products which comprises adding to the 15 product to be treated a soap which is substantially insoluble in water to facilitate the removal of wax at low temperatures, chilling the resultant mixture, and removing the wax from said product.

7. The method of removing wax from petroleum products which comprises adding to the petroleum product a soap which is substantially insoluble in water to facilitate the removal of wax at low temperatures, diluting the product with a 25 low boiling point hydrocarbon oil, chilling the resultant mixture to a temperature between 10° above zero F. and about 45° below zero F., subjecting the chilled mixture to centrifugal force to remove the wax, and removing said low boiling point hydrocarbon oil from said product.

8. The method of removing crystal-forming wax from petroleum oils which comprises adding to the oil to be treated a diluent and a soap which is substantially insoluble in water and which will 35 affect the structure of the wax at low temperatures to facilitate the removal of wax in a centrifuge, chilling the resultant mixture to a relatively low temperature, subjecting the chilled mixture to centrifugal force to remove wax, and 40 removing the diluent from said oil.

9. In the manufacture of low pour point lubricating oil from wax-containing mineral oils, the steps which comprise forming a mixture of a solvent, an oil containing wax and a small amount 45 of aluminum stearate, chilling the mixture to precipitate the wax and separating the precipitated wax from the oil by centrifuging.

HARRY T. BENNETT.

50